

# UNITED STATES PATENT OFFICE.

PORTER W. SHIMER, OF EASTON, PENNSYLVANIA.

## CASE-HARDENING OF METALS.

1,279,458.

Specification of Letters Patent. Patented Sept. 17, 1918.

No Drawing.

Application filed January 3, 1918. Serial No. 210,177.

*To all whom it may concern:*

Be it known that I, PORTER W. SHIMER, a citizen of the United States, residing at Easton, in the county of Northampton, State of Pennsylvania, have invented certain new and useful Improvements in Case-Hardening of Metals, (Case B;) and I do hereby declare the following to be a full, clear, and exact description of the invention, such as will enable others skilled in the art to which it appertains to make and use the same.

In an application for Letters Patent of the United States Serial Number 210,176, filed January 3, 1918, I have described and claimed the case-hardening of metals (for instance, articles of iron or steel) by means of a liquid melt or bath of fused salts (for instance, alkaline chlorids, chlorids of the alkaline earths, or alkaline chlorids and alkaline carbonates) which bath has been brought in contact with calcium cyanamid,—preferably by immersing the calcium cyanamid in the bath, in lump form and unchanged by atmospheric exposure.

As explained, in said co-pending application, the use of calcium cyanamid, in the more or less air-slaked condition in which it usually appears on the market, is attended with the disadvantage that persistent over-flowing frothing of the bath ensues,—probably due, in part at least, to the presence of moisture in the air-slaked cyanamid.

So also, when powdered or pulverulent calcium cyanamid is introduced, as such, into the melt, each individual particle of the cyanamid is chemically acted upon with a number of great disadvantages. The first is a voluminous and persistent frothing or foaming. The second disadvantage is that, by the occasional necessary addition of fresh cyanamid, the melt finally becomes so thickened by the accumulating cyanamid mud as to become useless. A third disadvantage is that a part of the case-hardening gases are generated and escape from the surface of the melt without coming in contact with the articles to be case-hardened.

I overcome these difficulties as will hereinafter more fully appear by imprisoning or combining the particles of the powdered calcium cyanamid in what may be called a coke-sponge. This hard sponge allows the liquid melt to penetrate, act upon, and leach out the case-hardening properties of the cyanamid, without any foaming. The coke-sponge also retains within its substance the

residuum which would otherwise constitute the cyanamid mud above referred to. This residuum is removed from the melt along with the spent coke in the basket. When alkaline chlorids alone are used in the melt, a large amount of case-hardening alkaline cyanid is formed in the bath, and the evolution of gas is only moderate. When the chlorids of the alkaline earths are present there is a much more lively evolution of gases and the case-hardening effects are correspondingly accelerated.

In carrying out the invention, air-slaked calcium cyanamid, if reduced to powder form, and also powdered calcium cyanamid generally, may be used to advantage, if the powdered cyanamid be first mixed with a suitable binder,—such as hard pitch (preferably pitch of such hardness that it can be pulverized and mixed with the powdered cyanamid, or of such a character that it can be ground to a pulverulent condition in the presence of the cyanamid). I have obtained good results by mixing three parts by weight of pulverized hard pitch with 7 parts of the powdered cyanamid, the mixture being effected in a revolving mixing cylinder.

The mixture of cyanamid and pulverized hard pitch (or other suitable liquid or solid binder capable of coking, such as tar) is then subjected to a red heat for the time necessary to drive off practically all of the volatile matter from the coked mass. After cooling, the coke-like mass is removed and broken into fragments of suitable size for use,—say 1 to 2 inches in diameter. The material, before coking, may also be formed into briquets of suitable size and shape for convenient use, though this is not necessary in order to obtain good case-hardening results.

The coke thus produced is introduced or brought into contact with the liquid melt of fused salts in the same manner described in my co-pending application hereinbefore referred to and performs the same function as the lumps or fragments of calcium cyanamid referred to therein, and without frothing.

The liquid melt or bath of fused salts into which the fragments of the coke-like mass of the present invention are to be immersed or otherwise brought in contact, may consist, for instance, of a fused mixture of sodium chlorid, calcium chlorid and barium chlorid, in equal proportions by weight, or a fused mixture of two parts of weight of

sodium chlorid to one part by weight of calcium chlorid, or of potassium chlorid, or of an easily fusible mixture of sodium and potassium chlorids. These mixtures are 5 typical of others of a similar character that may be employed as the liquid melt into which the fragments of the coke-like mass of calcium cyanamid and binder are to be introduced. For instance, alkaline carbonates may be added in making up the liquid melt.

The introduction of the fragments of the coke-like mass takes place to particular advantage if the fragments are placed in a 15 basket of iron wire, said basket being suspended in the liquid melt at a location near the bottom of the case hardening pot and in such manner as not to interfere with the use of the bath for the carrying on of the 20 case-hardening operation. The articles to be case-hardened are preferably suspended in the bath, as in the usual practice, upon suitable sustaining grids or the like, so as to be subjected to the best advantage to the 25 action of the bath.

Ordinarily, some time is necessary for the action of the bath upon the cyanamid contained in the fragments of the coke-like mass, in order to develop in the bath the 30 case-hardening properties. This time will vary from a few minutes up to say one-half hour or more, according to the size of the bath. The readiness of the bath to do case-hardening effectively is indicated by a 35 greater or less evolution of the gas from the bath. As soon as the gas begins to be actively evolved, the articles to be treated may be suspended in the bath, according to the usual practice, and for the period of 40 time desired. The case-hardening properties of the bath are best conserved by keeping the pot covered when not in use for case-hardening.

I have found that it is not necessary to 45 leave the basket containing the fragments of the coke-like mass continuously in the bath, but that after the removal of the basket and its contents, the bath retains its case-hardening properties for a considerable time. As indicated by a less lively evolution of the gas from the bath, when the alkaline earth chlorids are contained in it, and eventually by a weakening of the case-hardening effect upon the articles to be 50 treated, the case-hardening strength of the bath may be renewed by again suspending the basket with its contents in the melt.

The quantity of the fragments of the coke-like mass containing the cyanamid employed 55 may be varied according to the size of the bath, the shape, size and character of the articles to be case-hardened, and other conditions, as will be appreciated by those

skilled in the case-hardening art. I have obtained good case-hardening results, in the 65 treatment of articles of iron and steel, by suspending a sufficient quantity of the fragments of the coke-like mass to make up 15 pounds of calcium cyanamid in a bath containing 300 pounds of the liquid melt, i. e., 70 approximately 5% of the weight of the bath. Fresh quantities of the fragments may be added to the basket, from time to time, so as to maintain its ability to give the required case-hardening properties to the melt. It 75 is advisable to keep the basket and its contents in a dry place, during the interval of its periods of immersion in the bath, so that the calcium cyanamid may not become moist by attracting water from the atmosphere. 80 It is also advisable to keep it dry and warm by hanging it over the bath for a short time before immersing it therein, in order to drive off any moisture which may be present in the cyanamid. The gas which is evolved 85 in the liquid melt by the action of the cyanamid, and whose evolution continues even after the cyanamid has been withdrawn from the melt probably contributes to the case-hardening properties of the bath to a 90 considerable degree.

The basket of iron wire hereinbefore referred to will, of course, have wide meshes so as to permit full and free access of the liquid melt to its interior, and it will also 95 have a like open mesh cover so as to prevent the fragments of the coke-like mass from tendency to rise to the surface of the bath, or to otherwise pass out of the basket.

What I claim is:

1. The method of making a coke-like mass adapted for use in the case-hardening of metals, which comprises mixing calcium cyanamid with a suitable binder and coking the mass; substantially as described.

2. The method of making a coke-like mass adapted for use in the case-hardening of metals, which comprises producing a mixture of powdered calcium cyanamid and hard pitch or other "cooking" binder, coking the mass, thereby driving off volatile gases and converting the mixture into a coherent body adapted to be molded or broken up into fragments of suitable size for use in a case-hardening operation; substantially as described.

3. As a new composition of matter, a coke-like mass comprising calcium cyanamid associated with a binder; substantially as described.

4. As a new composition of matter, a coke-like mass, comprising calcium cyanamid associated with a coked pitch or tar; substantially as described.

In testimony whereof I affix my signature. 125  
PORTER W. SHIMER.

It is hereby certified that in Letters Patent No. 1,279,458, granted September 17, 1918, upon the application of Porter W. Shimer, of Easton, Pennsylvania, for an improvement in "Case-Hardening of Metals," errors appear in the printed specification requiring correction as follows: Page 1, line 112, the word "of" should read *by*; page 2, line 10, for the word "my" read *may*; same page, line 110, claim 2, for the word "cooking" read *coking*; and that the said Letters Patent should be read with these corrections therein that the same may conform to the record of the case in the Patent Office.

Signed and sealed this 29th day of October, A. D., 1918.

[SEAL.]

R. F. WHITEHEAD,  
*Acting Commissioner of Patents.*

Cl. 148—25.